

H. B. LAYMAN,  
BUILT-UP SHEET METAL STRUCTURE,  
APPLICATION FILED MAY 23, 1917.

1,418,309.

Patented June 6, 1922.



Fig. 1

WITNESSES:

*W. A. Kosken  
A. Bakelaar*



Fig. 2

INVENTOR.

*Hebron Bernard Layman*

# UNITED STATES PATENT OFFICE.

HEBON BERNARD LAYMAN, OF BRONXVILLE, NEW YORK.

## BUILT-UP SHEET-METAL STRUCTURE.

1,418,309.

Specification of Letters Patent. Patented June 6, 1922.

Application filed May 23, 1917. Serial No. 170,416.

To all whom it may concern:

Be it known that I, HEBON BERNARD LAYMAN, a citizen of the United States, residing at Bronxville, in the county of Westchester, State of New York, have invented certain new and useful Improvements in Built-Up Sheet-Metal Structures, of which the following is a full, clear, and exact description.

10 This invention relates to built-up structures, especially of sheet metal, such as pistons, crank shafts, or to connecting rods (for example of the type disclosed in U. S. Letters Patent No. 1,176,302), having bonded, 15 welded, fused or integrated therewith a thin non-ferrous metal sleeve, forming a journal or bearing, and composed of such an alloy of metals that it will have good bearing properties, and will retain these properties 20 when operated at relatively high temperatures; will be very ductile, hard, tough, take a high polish, and be of such high tensile strength, elongation and reduction, that it can be used in the form of very thin bushings. Also, that it will have a high melting 25 temperature, approaching that of steel, so that it can be welded or fused to, or integrated with, steel or iron, especially by the process described by me in my co-pending 30 application No. 168,514, entitled Immersion welding.

In the practice of my improved process of welding, I secure together two or more metal parts, joining the to-be-welded surfaces of the parts, (for example the sheet metal parts of the connecting rod disclosed in U. S. Letters Patent No. 1,176,302) by spot-welding, riveting, or in any other desirable way, and I then immerse the assembled parts in the molten alloy of metals at a 40 temperature approximating the melting point of the parts to be welded or integrated.

Having prepared a molten alloy of non-ferrous metals, which alloy, for example, 45 comprises relatively large proportions of copper, zinc and nickel, with a small content of magnesium, aluminum or manganese, which is added as a purifying agent to free the occluded gases and also to harden the 50 alloy, I then cover this molten alloy with a suitable flux; for example, one part calcium chloride, and two parts calcium fluoride, thus keeping the oxygen of the air from contact with the metal. Then, into this flux-covered molten alloy with its content of 55 nickel, the temperature of which approxi-

mates or exceeds the melting point of the article to be welded, I immerse or dip the assembled parts. It is commonly known that the melting point of steels ranges from about 2350 degrees F. to about 2580 degrees F., so when I immerse the assembled to-be-welded parts in the molten alloy, I do not allow them to remain therein long enough to reach the melting temperature of the steel. 60 The determination of the time to allow the assembled parts to remain in the alloy and the judging of the time that they remain therein, are both matters requiring great skill. I prefer to do the pre-heating, if any 65 is required, and the immersing and the subsequent quenching and reheating by positively timed mechanical means, rather than by hand.

On removing the structure from the alloy 70 and without affording it a chance to cool, it is shaken to remove any surplus metal. Thereafter, it is allowed to cool to the desired quenching temperature, which generally means a drop in temperature, of some 80 hundreds of degrees F., and with thin-walled structures as in the examples cited, this occurs rapidly. It is then plunged into oil, water or brine, as may be necessitated. Thereafter, if desired, it may be reheated 85 and quenched again, and some "heat-treatments" require the structure to be reheated a second time and "tempered" or "drawn back." As is well known, the number of times the article is reheated and quenched 90 depends upon the kind of material used, and the service to which the article is to be put. But, in any event, the welding alloy is such that the article may be reheated and quenched at any desired temperature any 95 number of times.

By way of example in the accompanying drawing, I show my invention as applied to such a sheet metal connecting rod, as is described in U. S. Patent No. 1,176,302, issued 100 to me March 21st, 1916.

Fig. 1 is a broken side elevation of an assembled pair of connecting rods;

Fig. 2 is a cross section on the vertical center line of Fig. 1.

In the accompanying drawing, in the two tines of the forked rod *a* is a steel backed and Babbitt-lined bushing *b* secured against rotation, and assembled thereon is a straight rod *c* which is free to oscillate. The details 110 of construction of this straight rod are disclosed in my co-pending application No.

159,398 filed April 3rd, 1917. In short, this rod is composed of two similar body sections  $c^1$  and an intermediate hard metal plate  $c^2$ . These three members are apertured in 5 one end to receive a piston pin; and secured to and uniting the several walls are flanged steel bushings or cuffs  $c^3$ , which constitute a piston pin boss, within which is a thin sleeve or bushing  $d$  of non-ferrous metal, for example, of the following analysis:

|           | Per cent. |
|-----------|-----------|
| Copper    | 69.5      |
| Nickel    | 29.00     |
| Magnesium | .5        |
| 15 Zinc   | 1.00      |

The melting temperature of this alloy is approximately equal to that of steel, whereas the ordinary bearing bronzes are of much 20 lower melting point than steel. The purpose of the content of nickel is to increase the melting temperature of the alloy and to toughen it. The purpose of the magnesium is to free the occluded gases, and the small 25 content of zinc is to render easier the rolling or extruding of the metal.

In practice, I prefer to roll the bearing metal alloy into strips, in which form it has a pronounced longitudinal grain structure, 30 then to cut the strips transversely into short lengths, and coil these lengths into tubes, so that the grain extends circumferentially of the tube, in which form the alloy possesses additional value as a bearing metal, but I 35 may draw or exclude the metal into tubes or cast or forge it.

In the course of making this rod  $c$  after the body sections  $c^1$  and the intermediate 40 plate  $c^2$  are formed and apertured, I assemble the flanged bushings  $c^3$  and within these fit the bearing  $d$ . I then use the bearing as a tubular rivet, spinning over the ends to secure the flanged bushings to the rod.

At the crank end of the rod are flanged 45 crank pin bushings  $c^4$  and a bearing metal liner  $e$ . These parts, though larger, correspond to the parts  $c^3$  and  $d$  of the piston end.

In the course of manufacture after all the 50 bushings are assembled with or upon the rod, the parts are fused together by im-

mersion in a molten alloy of metals, and subsequently heat-treated. By this process the bearings  $d$  and  $e$  are integrated with the sheet metal parts composing the rod. This 55 process is the subject of my co-pending application No. 168,514, filed May 14th, 1917, and is not here claimed by me.

In the construction shown, by fusing or integrating the bearing  $d$  with the rod, I am 60 able to use a very thin bearing metal sleeve, which for this service need not exceed from .005" to .030" in thickness, depending upon the service, and generally I prefer .015" 65 thick.

In such a structure as a connecting rod or piston or crank shaft of a high-speed gas-engine, the dissipation of the heat generated in the bearings is a very important factor. By my construction I obtain an integral 70 strong head-end structure for the connecting rod shown, small and light as possible, and having the ability to radiate heat rapidly.

Having fully described my invention, what I claim as new and desire to secure by Letters Patent, is:

1. A built-up sheet ferrous metal structure having integrated therewith a tubular non-ferrous metal bearing, in which the grain structure is circumferential of the 80 bearing.

2. A built-up sheet metal structure having fused thereto a sleeve of non-ferrous sheet bearing metal, the metal of the bearing having substantially the same melting point as 85 the metal of the structure.

3. A sheet metal structure having integrated therewith a bearing formed of an alloy comprising a relatively large proportion of copper and a constituent which will 90 raise the melting point, in which the grain structure is circumferential of the bearing.

4. A ferrous metal connecting rod, or the like, having a cylindrical aperture lined with non-ferrous metal which is permanently 95 bonded or unified therewith, the metal of the lining having substantially the same melting point as the metal of the connecting rod.

In testimony whereof I affix my signature. 100

HEBON BERNARD LAYMAN.